

# United States Patent Office

3,070,436

Patented Dec. 25, 1962

1

3,070,436

## METHOD OF MANUFACTURE OF HOMOGENEOUS COMPOSITIONS

Bernard H. Trifileman, Fair Lawn, N.J., assignor to Curtiss-Wright Corporation, New York, N.Y., a corporation of Delaware

No Drawing. Filed Mar. 17, 1959, Ser. No. 799,855

11 Claims. (Cl. 75—0.5)

The present invention relates to a method for manufacturing homogeneous compositions of several elements, and in particular to the production of homogeneous compositions of dispersions of a metal phase and oxides of finite size, in alloys, cermets and ceramics. This is a continuation-in-part of my earlier filed application Serial No. 566,767, filed February 21, 1956, and entitled Method of Manufacture of Homogeneous Compositions, now Patent No. 2,893,859, issued July 7, 1959.

In accordance with my copending application, there was provided a method of preparing a homogeneous composition of several elements by starting with a homogeneous solution of the several elements in a volatile solvent. The term "solution" included true solutions and colloidal suspensions. The solution of the several elements was dried under conditions appropriate to drive off substantially all of the volatile solvent, without causing segregation of the several elements. The drying action, which was characterized as "quick-drying," formed a homogeneous molecular mixture of the several elements in solid form, which by further treatment, could be reduced to attain a molecular mixture in powdered form or a regulus alloy. Although the method of my copending application had numerous and substantial uses, at times the requirement is imposed that material, in the form of finite size particles, is to be uniformly dispersed in a matrix of an atomic mixture of the several elements of the alloy, cermet or ceramic mixture. Illustrative of this requirement is the need to disperse uranium oxide uniformly in stainless steel or other similar corrosion-resistant metals for use in nuclear reactors. Further, the process of my copending application can be used only in the production of alloy powders which can be produced from mixed oxides below the melting temperature of the desired alloy and below the temperature at which the one or more elements of the alloy would melt and separate from the remaining oxides. As a practical matter, powders of alloys containing reactive metals such as aluminum, titanium and columbium were difficult, if not impossible, to manufacture by the disclosed process of said copending application. Still further to arrive at an alloy or cermet of a particular composition, it was essential to practice the entire process, including the several steps thereof. As a practical matter, it was not possible to prepare a standard or basic alloy of a prescribed composition; and then by the addition of materials thereto alter the composition to create a different, but somewhat related alloy. The practice of the complete process requires the initial set-up of the equipment for the manufacture of the particular alloy under consideration, followed by the task of cleaning out the equipment before beginning to process a different alloy. Consequently, from the cost standpoint, alloys or cermets which are not in too great demand were rather expensive to manufacture due to the need of a complete and separate manufacturing cycle.

Broadly, it is an object of the present invention to provide an improved process for the manufacture of homogeneous compositions which obviates one or more of the aforesaid difficulties.

It is a further object of the present invention to provide a method for the manufacture of homogeneous compositions of a dispersion of a metal phase and oxides of

2

finite size in alloys, cermets and ceramics wherein the metal phase is uniformly dispersed in a matrix of such alloys, cermets or ceramics.

It is a still further object of the present invention to provide a method for the production of alloy metal powders and cermets from reactive metals, including without limitation aluminum, titanium and columbium.

A still further object of the present invention is to provide a method which facilitates the initial fabrication of an alloy metal powder, with the facility to convert such alloy metal powder to a related alloy containing further metals and/or a different composition.

A further problem which may be presented in the production of true alloy powders is the difficulty of working such powders into usable forms and shapes. Frequently, such true alloy powders are exceptionally hard and brittle such that the particles do not yield or interlock in press-type operations. This consequently precludes the briquetting of such powders into parts and/or the rolling of such powders into strips of materials. Typical alloy powders which are not readily worked due to their hardness or brittleness are Alnico V and Renet 21. Further, very few fabricating plants are equipped to manufacture powdered metal parts by pressing such powdered metals and heating the resulting green compact, which coupled with the difficulty in the first instance of making certain parts by this technique, points to the need for the facility to convert alloy powder into strip form. With the conversion of such alloy powders into strips of material, new fields of use for alloy metal powders become available. Certain materials cannot be readily fabricated by conventional techniques. Specifically, some of these materials are rather expensive to fabricate (e.g. thin gauge Inconel X). Others are rather difficult to fabricate (e.g. Renet 21) and still others are virtually impossible to fabricate (e.g. cermets and alloy and cermet-dispersions).

Accordingly, it is a further object of the present invention to provide an improved method for manufacturing alloy powders which have characteristics making it readily possible to fabricate such alloy powders, and advantageously roll certain of these alloy powders into strip form. Specifically, it is within the scope of this invention to fabricate by powder metallurgy techniques materials which heretofore were difficult, virtually impossible and extremely expensive to fabricate.

In accordance with illustrative method aspects of the present invention, there is provided a method for the manufacture of homogeneous compositions of dispersions of a metal phase and oxides of finite size in alloys, cermets and ceramics which comprises the steps of preparing a homogeneous solution of the several elements in the composition in a volatile solvent including constituents selected from the group consisting of nitric acid, sulphuric acid, ammonia and water. The term "solution" in the instant application is intended to include dispersions of finite particles. The phase to be dispersed is added in solid form to the solution and the resultant solution-dispersion is blended until a uniform system is achieved. The solution-dispersion is then subjected to quick drying to drive off a substantial amount of the volatile solvent under conditions selected to preclude segregation of the several elements and to assure the formation of a homogeneous molecular mixture of the several elements surrounding a homogeneous dispersion of the phase in solid form.

By this improved process alloy metal powders, cermets and ceramics can be produced which comprise a continuous phase of a homogeneous atomic or molecular mixture of elements with a homogeneous dispersion of a second phase of finite size, such as an oxide. Examples of the alloy metal powders which can be made include, without

limitation, stainless steel with uranium oxide as a dispersed phase and monel-five percent aluminum oxide with a dispersed phase of thorium oxide.

In accordance with further method aspects of the present invention, it is possible to initially manufacture a homogeneous composition of a basic alloy metal and/or ceramic by preparing a homogeneous solution of the requisite composition in a volatile solvent, including constituents selected from the group consisting of nitric acid, sulphuric acid, ammonia and water, with the solution being subjected to quick drying under conditions to preclude segregation of the several elements and to assure the formation of a homogeneous molecular mixture of the several elements in solid form. The mixture is then treated to obtain a reduced powder and the reduced powder may be heated in the presence of a powdered alloy of unreduceable and/or additional metals to effect further alloying to obtain a desired end composition. As an example of this, a 304 stainless steel may be made according to my process, and by the addition of ferromolybdenum, such 304 stainless steel may be converted to 316 stainless steel. Further illustrating this conversion, Alnico V mixing alloy may be treated with ferro aluminum to achieve a workable Alnico V powder. Still further, 4600 steel may be changed to 4650 steel powder by adding lampblack to the 4600 steel. The conversion of the basic alloy powder may be readily accomplished by mixing or blending such alloy powder with the additional alloying agent, preferably being of a finer size, under a controlled atmosphere for a prescribed time and at a prescribed temperature in accordance with the materials under consideration.

The following examples will illustrate the manner in which the present invention may be employed to practice the manufacture of homogeneous compositions, but it is to be expressly understood that the invention is not limited to these illustrative examples:

#### EXAMPLE I

90% 304 Stainless Steel-10% Aluminum Oxide (Continuous Phase), 90% by weight; Zirconium Dioxide, 20-25 microns average size (Dispersed Phase), 10% by weight

(1) 63 parts iron, 9 parts nickel, and 15.3 parts



were dissolved in excess nitric acid; 36 parts chromic acid were dissolved in a little water and the solutions were mixed and concentrated to a boiling point of 118° C. To the concentrated solution was added 11 parts of zirconium dioxide of a size of 20-25 microns. The solution-dispersion was mixed in a blender until a uniform system was achieved.

(2) The resulting solution-dispersion was fed dropwise, while being stirred, onto a hot metal surface maintained at 300° C. and left there for 30 seconds whereupon a substantial amount of the volatile solvent distilled. A solid homogeneous product resulted.

(3) This product was heated at 800° C. for 20 minutes to remove the remainder of the volatiles.

(4) The homogeneous product was ground in a hammer mill until the particles all passed a screen of 100 mesh.

(5) The powder was then reduced in a tube furnace under a hydrogen atmosphere at 1000° C. for 60 minutes. 90% of the oxygen was removed from the iron, nickel, and chromium oxides.

(6) The resulting powder was deagglomerated and mixed with a stoichiometric amount of lampblack to reduce the remaining oxides of chromium-iron-nickel to carbon monoxide.

(7) The powder was then further reduced at 1150° C. for 30 minutes under a low flow of hydrogen.

(8) The product was deagglomerated and the resulting powder was non-magnetic, corrosion resistant to nitric

acid, sponge-like in structure, and contained no carbon. This powder was easily pressed under normal powder metallurgy pressures and showed good strength after sintering. The powders were able to be easily rolled into strip form and exhibited after sintering both the formability of metals and the heat stability of ceramics.

#### EXAMPLE II

##### Alnico V Powder and Strip

(1) Alnico V mixing alloy powder of a size finer than 100 mesh and of a composition of 28.6% Co, 3.6% Cu, 51.2% Fe and 16.5% Ni was made according to the general procedure detailed in my copending application. 336 parts of this powder was mixed with 64 parts of a 50% Al, 50% Fe powder of a size finer than 325 mesh. The powder was heated in a rotary kiln at 875° C. for 30 minutes under a hydrogen atmosphere. The powders had sintered slightly but were easily broken up to finer than 100 mesh. The powder, a partially alloyed Alnico V material, had a composition of 8% Al, 24% Co, 3% Cu, 51% Fe, and 14% Ni. This powder was able to be pressed and sintered, and the sinterings showed higher density and better sintered properties than a similar part made from primary powders. Further, the powder was fed to a rolling mill with horizontal rolls and a green strip obtained which was of the order of 0.035 inch thick. This strip was sintered at 900° C. for one hour under hydrogen and was then rolled down to 0.020 inch. The strip was then resintered at 900° C. for one hour and re-rolled to 0.010 inch.

For comparison purposes, an alloyed powder was made by grinding cast Alnico and it was attempted to press and roll bond this Alnico powder. In both operations, the powders could not be compacted to the desired shapes.

#### EXAMPLE III

##### Steel Powder, AISI 4650

An AISI 4600 steel powder of a size finer than 100 mesh and of a composition of 97.75% Fe, 2.0% Ni and 0.25% Mo was made according to the general procedure detailed in my copending application. This powder, when tested by being pressed at 40 tons per square inch followed by sintering at 1150° C. for one hour under hydrogen, was found to have a tensile strength of 30,000 p.s.i. and an elongation of 15%. 99.5 parts of this 4600 steel powder was then mixed with 0.55 part lampblack and heated at 750° C. in a rotary kiln for 30 minutes under a hydrogen atmosphere. The resulting powder had sintered slightly and was easily broken up to a size finer than 100 mesh. This powder, a 4650 steel powder, when tested as the 4600 steel powder, showed a tensile strength of 79,000 p.s.i. and an elongation of 2.9%.

#### EXAMPLE IV

##### Renet #21, Powder and Sheet

A Renet 21 mixing alloy powder of a size finer than 100 mesh and of a composition of 12.4% Co, 20.9% Cr, 11.0% Mo, and 55.7% Ni was made according to the general procedure detailed in my copending application. 91 parts of this alloy was mixed with 6 parts of a 50% Ni, 50% Ti powder, 3 parts of a 50% Ni, 50% Al powder and 0.13 part of lampblack, the latter powders all being finer than 325 mesh. The powders were heated in a tube furnace at 900° C. under a hydrogen atmosphere for one hour. The powders were sintered slightly, but were easily broken up to a size finer than 100 mesh. The powder, a partially alloyed Renet 21, had a composition of 1.5% Al, 0.12% C, 11.3% Co, 19% Cr, 10% Mo, 3% Ti and the balance Ni.

This powder was able to be easily pressed and sintered; and the green bar showed excellent handling strength and the sintered bar showed excellent tensile strength. Further, this powder was fed to a rolling mill, with horizontal rolls and a green strip of the order of 0.034 inch thick

with excellent handling strength was obtained. This strip was sintered at 1100° C. for one hour under a low flow of hydrogen and was then rolled in a two-high vertical mill to 0.019 inch thick. The resulting strip was heated at 1200° C. for one hour under a low hydrogen flow and then rerolled to 0.010 inch in a two-high vertical mill. The resulting strip was found to have excellent strength.

## EXAMPLE V

## 90% Stainless Steel-10% Aluminum Oxide Cermet in Strip Form

A 90% 304 stainless steel-10%  $\text{Al}_2\text{O}_3$  cermet powder of a size finer than 100 mesh was made according to the general procedure detailed in my copending application. This powder was fed to a rolling mill with horizontal rolls and a green strip 0.020 inch thick and with good handling strength obtained. This strip was sintered at 1200° C. for one hour under a hydrogen atmosphere. The strip was then rolled down to 0.010 inch and showed good room temperature strength coupled with excellent high temperature strength.

What I claim is:

1. A method for manufacturing homogeneous compositions of several elements including at least one metal and a dispersed oxide phase of finite particle size in alloys, cermets and ceramics comprising the steps of preparing a homogeneous solution of the several elements in the composition in a volatile solvent including constituents selected from the group consisting of nitric acid, sulfuric acid, ammonia, and water, adding said oxide phase to be dispersed in solid form to said solution and blending the resultant solution-dispersion, subjecting said solution-dispersion to quick drying to drive off a substantial amount of said volatile solvent under conditions selected to preclude segregation of said several elements and to assure the formation of a homogeneous molecular mixture of said several elements surrounding a homogeneous dispersion of said oxide phase in solid form, reducing said mixture to obtain a powder with a homogeneously dispersed phase of finite size, and rolling said powder to obtain a strip of material.

2. The method according to claim 1 including the further step of heating said strip under a controlled atmosphere for a time period in the range of 10 to 120 minutes and at a temperature in the range of 500° C. to 1500° C.

3. In a method for manufacturing homogeneous compositions of alloy metals and cermets, the steps of preparing a homogeneous solution of the several elements in the composition in a volatile solvent including constituents selected from the group consisting of nitric acid, sulfuric acid, ammonia and water, subjecting said solution to quick drying to drive off a substantial amount of said volatile solvent under conditions selected to preclude segregation of said several elements and to assure the formation of a homogeneous molecular mixture of said several elements in solid form, treating said molecular mixture to obtain a powder and reducing said powder, and heating said powder with another alloy powder of a finer size under a controlled atmosphere for a time period in the range of 10 to 120 minutes and at a temperature in the range of 500° C. to 1500° C.

4. In a method for manufacturing homogeneous compositions of alloy metals and cermets, the steps of preparing a homogeneous solution of the several elements in the composition in a volatile solvent including constituents selected from the group consisting of nitric acid, sulfuric acid, ammonia and water, subjecting said solution to quick drying to drive off a substantial amount of said volatile solvent under conditions selected to preclude segregation of said several elements and to assure the formation of a homogeneous molecular mixture of said several elements in solid form, further heating said molecular mixture to drive off any residue of said volatile solvent, treating said molecular mixture to obtain a powder and reducing said powder, heating said powder with an-

other alloy powder of a finer size under a controlled atmosphere for a time period in the range of 10 to 120 minutes and at a temperature in the range of 500° C. to 1500° C., and rolling the resultant powder to obtain a strip of material.

5. In the method according to claim 4, the further step of heating said strip under a controlled atmosphere for a time period in the range of 10 to 120 minutes and a temperature in the range of 500° C. to 1500° C.

10 6. In a method for manufacturing homogeneous compositions of alloy metals and cermets, the steps of preparing homogeneous solution of the several elements in the composition in a volatile solvent including constituents selected from the group consisting of nitric acid, sulfuric acid, ammonia and water, subjecting said solution to quick drying to drive off a substantial amount of said volatile solvent under conditions selected to preclude segregation of said several elements and to assure the formation of a homogeneous molecular mixture of said several elements in solid form, further heating said molecular mixture to drive off any residue of said volatile solvent, treating said molecular mixture to obtain a powder and reducing said powder, and rolling said powder to obtain a strip of material.

20 7. In the method according to claim 6, the further step of heating said strip under a controlled atmosphere for a time period in the range of 10 to 120 minutes and at a temperature in the range of 500° C. to 1500° C.

25 8. A method for manufacturing homogeneous compositions of alloys, cermets, and ceramics having dispersed therein oxide of finite size, comprising the steps of preparing a homogeneous solution of the several elements in the composition in a volatile solvent including at least one constituent selected from the group consisting of nitric acid, sulfuric acid, ammonia, and water; adding to said solution an oxide of finite particle size and insoluble in said solvent and blending the resultant solution-dispersion; and subjecting said solution-dispersion to quick drying to drive off a substantial amount of said volatile solvent under conditions selected to preclude segregation of said several elements and to assure the formation of a homogeneous molecular mixture of said several elements homogeneously surrounding a dispersion of said finite-sized oxide particles.

30 9. A method for manufacturing homogeneous compositions of alloys, cermets, and ceramics having dispersed therein oxide of finite size, comprising the steps of preparing a homogeneous solution of the several elements in the composition in a volatile solvent including at least one constituent selected from the group consisting of nitric acid, sulfuric acid, ammonia, and water; adding to said solution an oxide of finite particle size and insoluble in said solvent and blending the resultant solution-dispersion; and subjecting said solution-dispersion to quick drying to drive off a substantial amount of said volatile solvent under conditions selected to preclude segregation of said several elements and to assure the formation of a homogeneously surrounding a dispersion of said finite-sized oxide particles, and reducing said mixture to obtain a powder with a homogeneously dispersed phase of finite size.

35 10. A method for manufacturing homogeneous compositions of alloys, cermets, and ceramics having dispersed therein oxide of finite size, comprising the steps of preparing a homogeneous solution of the several elements in the composition in a volatile solvent including at least one constituent selected from the group consisting of nitric acid, sulfuric acid, ammonia, and water; adding to said solution an oxide of finite particle size and insoluble in said solvent and blending the resultant solution-dispersion; and subjecting said solution-dispersion to quick drying to drive off a substantial amount of said volatile solvent under conditions selected to preclude segregation of said several elements and to assure the formation of a homogeneous molecular mixture of said

several elements homogeneously surrounding a dispersion of said finite-sized oxide particles, reducing said mixture to obtain a powder with a homogeneously dispersed phase of finite size, and then heating said powder with another alloy powder of a finer size under a controlled atmosphere for a time period in the range of 10 to 120 minutes and a temperature in the range of 500° C. to 1500° C.

11. A method for manufacturing homogeneous compositions of several elements including at least one metal and a dispersed oxide phase of finite particle size in alloys, cermets, and ceramics comprising the steps of preparing a homogeneous solution of the several elements in the composition in a volatile solvent including constituents selected from the group consisting of nitric acid, sulfuric acid, ammonia and water, adding said oxide phase to be dispersed in solid form to said solution, and blending the resultant solution-dispersion, subjecting said solution-dispersion to quick drying to drive off a substantial amount of said volatile solvent under conditions selected to preclude segregation of said several elements and to assure

the formation of a homogeneous molecular mixture of said several elements surrounding a homogeneous dispersion of said oxide phase in solid form, reducing said mixture to obtain a powder with a homogeneously dispersed phase of finite size, and then heating said powder with another alloy powder of a finer size under a controlled atmosphere for a time period in the range of 10 to 120 minutes and a temperature in the range of 500° to 1500° C.

10

## References Cited in the file of this patent

## UNITED STATES PATENTS

|           |            |               |
|-----------|------------|---------------|
| 1,319,589 | Jones      | Oct. 21, 1919 |
| 2,406,172 | Smithells  | Aug. 20, 1946 |
| 2,893,859 | Triffleman | July 7, 1959  |

## FOREIGN PATENTS

|         |               |              |
|---------|---------------|--------------|
| 784,153 | Great Britain | Oct. 2, 1957 |
|---------|---------------|--------------|

20